

## UNITED STATES PATENT OFFICE

PASCAL J. MORELL, OF WATERBURY, CONNECTICUT, ASSIGNOR TO THE AMERICAN BRASS COMPANY, OF WATERBURY, CONNECTICUT, A CORPORATION OF CONNECTICUT

## ZINC BASE ALLOY

No Drawing.

Application filed June 18, 1930. Serial No. 462,141.

This invention relates to zinc base alloys, and more particularly to such alloys for die casting and the like. At the present time zinc base alloys suitable for die casting and known 5 and in extensive use, and under favorable conditions have a comparatively high tensile strength, relatively high impact strength and fair ductility. A zinc base die casting alloy commonly in use at the present time contains about 4% aluminum, about 3% copper, about 10 0.1% magnesium, and the balance zinc. It is widely used in the die casting industry. Tests have shown, however, that the strength of this alloy, like all other known zinc base 15 alloys, decreases with time after casting. The decrease in physical properties is particularly marked if the cast alloy is heated in the presence of water vapor. This and other known zinc base alloys are subject to a certain 20 inter-crystalline oxidation or corrosion in the presence of warmth and moisture, causing swelling, warping and loss of strength. Still further, changes occur in these alloys upon aging at the ordinary temperatures 25 unaccompanied by serious inter-crystalline oxidation, which changes may result in serious loss or decrease of certain physical properties of the alloy, such as tensile and impact strength.

It is, therefore, an object of this invention 30 to produce an improved zinc base alloy which is adapted to be cast in permanent and sand molds, and is also especially adapted for die casting. A particular object is to produce an 35 improved alloy which is not subject to inter-crystalline corrosion or at least in which this corrosion is greatly decreased, and especially in which the corrosion attack in the presence of moisture and heat is greatly decreased and 40 practically eliminated.

It is also an object of the invention to produce an alloy in which deterioration in strength is less than in the known alloys, and in which the change in physical properties as 45 measured by tensile strength, elongation and impact value is small, thus making it particularly valuable for die casting and similar purposes.

The invention involves the addition of a 50 hardener such as silicon in comparatively

small amounts to zinc base alloys and more particularly to a zinc base alloy containing copper. I have found that silicon when added to zinc base copper alloys produces an alloy which is very resistant to deterioration by 55 corrosion even under adverse conditions of heat and moisture, and furthermore, produces an alloy which is not subject to undesirable changes in physical properties or to structural or equilibrium changes.

Silicon can be used alone with the zinc and copper or in combination with any of the following metals such as manganese, magnesium, nickel, iron, cobalt or chromium. The silicon alone has a hardening effect and 60 gives improved physical properties to the zinc base copper alloy, but it is desirable under certain conditions in addition to silicon to add one or more of the other metals to the zinc base copper alloy. Zinc base alloys containing copper, particularly from about 1 to 65 about 15 percent of copper, are greatly improved by the presence of silicon from approximately .005 to about 5%, and the alloy may be further improved by the addition of 70 small amounts of magnesium, manganese, nickel, iron, cobalt or chromium as further described. Such alloys have high tensile 75 strength and are much less subject to corrosion, and particularly are more resistant to corrosion in the presence of warmth and moisture than heretofore known zinc base alloys. Furthermore, aging or deterioration 80 in physical properties such as tensile and impact strength when unaccompanied by corrosion, is much less in these alloys.

A further reason for adding magnesium is its effect in reducing or eliminating the deleterious effect of impurities such as lead which may be present in commercial grades of zinc.

The presence of aluminum is of further advantage if the alloy is to be used for die casting due to its action in preventing the attack of the zinc on the iron and steel of the dies or other parts of the die casting equipment.

These zinc base alloys are predominately zinc and contain from about 1 to about 15% copper and relatively small amounts of silicon. To these alloys may be added any of 100

the other metals above mentioned. The silicon is preferably from about .08 to about .15%, but may vary from about .005 to about 5%. When aluminum is added it is preferably from about .25 to about .35%, but may vary from about .005 to about 10%. The manganese is preferably from about .035 to about .045%, but may vary from about .005 to about 5%. The percentage of magnesium is preferably from about .02 to about .03%, but may vary from about .001 to about 2%.

That is, the present preferred alloy is a zinc base alloy containing about 2.5 to about 3.5% copper; about .25 to about .35% aluminum; about .08 to about .15% silicon; about .035 to about .045% manganese, and about .02 to about .03% magnesium.

Other percentages within the limits given will produce alloys having improved physical properties and are useful alloys, but the specific preferred alloy mentioned appears to have the best physical properties, especially for die casting, and seems to retain these properties with the least deterioration either by ordinary ageing or by corrosion in the presence of heat and moisture. Thus, an alloy containing approximately .32% aluminum; 2.91% copper; .10% silicon; .023% magnesium; and .04% manganese was found on test to have zero expansion or at least less than .0002 inches expansion on a six inch specimen after exposure to water vapor for ten days at 95 degrees C. The tensile strength as cast was about 32,300 pounds per square inch, and after exposure to water vapor and heat for ten days at 95 degrees C. was about 27,530 pounds per square inch. Elongation as cast was about 1.38% and after exposure as specified .88%. With the Charpy type of impact test it showed an impact strength of 31.6 foot pounds per square inch as cast, and after exposure as specified 18.7. It also had good casting characteristics.

As a result of my investigations, I have found that the percentages of silicon substantially as specified in the zinc base copper alloys produces an alloy with increased resistance to inter-crystalline corrosion. The effect of the silicon alone is not as great as when used with one or more of the other elements as specified. In other words, if we leave out the magnesium, for example, in the specific preferred alloy above mentioned, we get a desirable alloy with good physical properties and small expansion, but by including the magnesium, the properties are improved still further and the expansion still further reduced or practically eliminated. It is further to be noted in all of the above mentioned zinc base copper silicon alloys containing manganese, that iron, chromium, cobalt and nickel may each be used as a substitute for the manganese, and would act similarly to the manganese. Investigations indicate that best results are secured

when in the zinc base copper alloy, or zinc base copper aluminum alloy, silicon, manganese, and magnesium are used, or some of the elements mentioned substituted for the manganese. I, therefore, wish it to be understood that in the claims specifying manganese with silicon I can substitute iron, chromium, cobalt or nickel in place of the manganese, and intend the claims to cover this.

In effect, the alloys of the invention have good casting properties, low shrinkage, practically no expansion and corrosion after exposure to heat and moisture, and deteriorate much less in physical properties as measured by strength, elongation, and impact value as compared with the now known zinc base alloys.

Having thus set forth the nature of my invention, what I claim is:

1. A zinc base alloy containing about 1 to about 15% copper, and about .005 to about 5% silicon.
2. A zinc base alloy containing about 1 to about 15% copper, about .005 to about 5% silicon, and about .005 to about 5% manganese.
3. A zinc base alloy containing about 1 to about 15% copper, about .005 to about 5% silicon, and about .001 to about 2% magnesium.
4. A zinc base alloy containing about 1 to about 15% copper, about .005 to about 5% silicon, and about .005 to about 10% aluminum.
5. A zinc base alloy containing about 1 to about 15% copper, about .005 to about 5% silicon, about .001 to about 2% magnesium and about .005 to about 5% manganese.
6. A zinc base alloy containing about 1 to about 15% copper, about .005 to about 5% silicon, about .001 to about 2% magnesium and about .005 to about 10% aluminum.
7. A zinc base alloy containing about 1 to about 15% copper, about .005 to about 5% silicon, about .005 to about 5% manganese, and about .005 to about 10% aluminum.
8. A zinc base alloy containing about 1 to about 15% copper, about .005 to about 5% silicon, about .001 to about 2% magnesium, about .005 to about 5% manganese, and about .005 to about 10% aluminum.
9. A zinc base alloy containing about 1 to about 8% copper, about .025 to about .3% silicon, about .01 to about .1% manganese, about .025 to about 1% aluminum and about .01 to about .25% magnesium.
10. A zinc base alloy containing about 1.5 to about 5% copper, about .05 to about .20% silicon, about .02 to about .05% manganese, about .05 to about .50% aluminum and about .01 to about .05% magnesium.
11. A zinc base alloy containing about 2.5 to about 3.5% copper, about 0.25 to about 0.35% aluminum, about .08 to about .15% silicon, and about .005 to about 5% manganese.

silicon, about .035 to about .045% manganese, and about .02 to about .03% magnesium.

12. A zinc base alloy containing approximately 3% copper, .30% aluminum, .10%  
5 silicon, .025% magnesium, and .04% manganese.

In testimony whereof I affix my signature.  
PASCAL J. MORELL.

10

15

20

25

30

35

40

45

50

55

60

65